

# United States Patent Office

3,116,145

Patented Dec. 31, 1963

1

3,116,145

**TUNGSTEN-HAFNIUM ALLOY CASTING**  
 Marion Semchyshen, Dearborn, Mich., assignor to American Metal Climax, Inc., New York, N.Y., a corporation of New York  
 No Drawing. Filed Apr. 30, 1962, Ser. No. 191,305  
 9 Claims. (Cl. 75—176)

The present invention relates to cast tungsten base alloys containing hafnium and which are characterized by the fact that they are capable of being worked at elevated temperatures and have unusually high strength and hardness at temperatures above 2000° F. This application is a continuation-in-part of applicant's copending application, Serial No. 41,766, filed July 11, 1960.

The alloys of the present invention are castings containing from .02% to 5% hafnium, up to .50% carbon. The balance consists essentially of tungsten except that small quantities of zirconium, tantalum, columbium or molybdenum may be present as optional ingredients. Thus, one or more of the elements of zirconium, tantalum and columbium may be present in amounts not exceeding a total of about 1% and molybdenum may be present in an amount not exceeding about 10%. Oxygen, even in the smallest amounts, is deleterious and hence must be less than .005% and preferably less than .001%.

Highly useful alloys within the scope of the present invention include alloys containing .01% to .10% carbon. However, when carbon is present in amounts in the order of .01% or more, the hafnium content should not exceed about 1%. Larger quantities of hafnium, within the limits stated above, may be present in carbon free alloys or alloys containing less than .01% carbon.

The alloys of the present invention may be prepared by arc-melting in vacuum, preferably using a furnace of the type disclosed in the United States Patent 2,656,743. A preferred method of deoxidizing the melt is by adding carbon to the charge to react with any oxygen present in raw materials and in quantities which will leave the desired excess in the final casting. The absolute pressure during the melting operation is preferably maintained below 50 microns of mercury.

The following are specific examples of alloys coming within the scope of the invention:

| Percent Hafnium | Percent Carbon | Percent Molybdenum | Percent Tungsten |
|-----------------|----------------|--------------------|------------------|
| 2.4             | -----          | -----              | Balance.         |
| 2.85            | -----          | -----              | Do.              |
| .45             | .002           | -----              | Do.              |
| 1.2             | .004           | -----              | Do.              |
| 2.8             | .007           | -----              | Do.              |
| .22             | .014           | -----              | Do.              |
| .47             | .006           | -----              | Do.              |
| .10             | .01            | 10                 | Do.              |
| .05             | .015           | -----              | Do.              |

2

All proportions given are proportions by weight.

What is claimed is:

1. A cast alloy containing from .02% to 5% hafnium, up to .50% carbon, less than .005% oxygen, not more than 1% of metal from the group consisting of zirconium, tantalum and columbium, not more than 10% molybdenum and the balance consisting essentially of tungsten.
2. A cast alloy containing from .02% to 1% hafnium, up to .50% carbon, less than .005% oxygen, not more than 1% of metal from the group consisting of zirconium, tantalum and columbium, not more than 10% molybdenum and the balance consisting essentially of tungsten.
3. A cast alloy containing from .02% to 1% hafnium, up to .10% carbon, less than .005% oxygen, not more than 1% of metal from the group consisting of zirconium, tantalum and columbium, not more than 10% molybdenum and the balance consisting essentially of tungsten.
4. A cast alloy containing from .02% to 5% hafnium, up to .50% carbon, less than .005% oxygen, not more than 10% molybdenum and the balance consisting essentially of tungsten.
5. A cast alloy containing from .02% to 1% hafnium, up to .50% carbon, less than .005% oxygen, not more than 10% molybdenum and the balance consisting essentially of tungsten.
6. A cast alloy containing from .02% to 1% hafnium, up to .10% carbon, less than .005% oxygen, not more than 10% molybdenum and the balance consisting essentially of tungsten.
7. A cast alloy containing from .02% to 5% hafnium, up to .50% carbon, less than .005% oxygen, and the balance consisting essentially of tungsten.
8. A cast alloy containing from .02% to 1% hafnium, up to .50% carbon, less than .005% oxygen, and the balance consisting essentially of tungsten.
9. A cast alloy containing from .02% to 1% hafnium, up to .10% carbon, less than .005% oxygen, and the balance consisting essentially of tungsten.

## References Cited in the file of this patent

### UNITED STATES PATENTS

|    |           |                      |               |
|----|-----------|----------------------|---------------|
| 45 | 2,234,969 | Hensel et al. -----  | Mar. 18, 1941 |
|    | 2,580,273 | Bens et al. -----    | Dec. 25, 1951 |
|    | 2,678,268 | Ham et al. -----     | May 11, 1954  |
|    | 2,678,269 | Ham et al. -----     | May 11, 1954  |
|    | 2,678,270 | Ham et al. -----     | May 11, 1954  |
| 50 | 2,678,271 | Ham et al. -----     | May 11, 1954  |
|    | 2,678,272 | Ham et al. -----     | May 11, 1954  |
|    | 2,798,808 | Iredell et al. ----- | July 9, 1957  |
|    | 2,947,624 | Semchyshen -----     | Aug. 2, 1960  |
|    | 2,977,225 | Wlodek et al. -----  | Mar. 28, 1961 |

### FOREIGN PATENTS

|           |                     |               |
|-----------|---------------------|---------------|
| 216,840   | Great Britain ----- | June 29, 1925 |
| 1,233,810 | France -----        | May 9, 1960   |

The alloys of the present invention may be forged or worked at temperatures in the neighborhood of 3600° F. to 4000° F.

55